

# United States Patent

[19]

Mertens et al.

[11] 3,820,995

[45] June 28, 1974

[54] **PHOTOCROMIC MATERIAL  
CONTAINING A SPIROPYRAN COMPOUND,  
A POLYHALOGENATED HYDROCARBON  
PHOTOACTIVATOR AND AN  
ACETANILIDE SENSITIZER AND THE USE  
THEREOF IN PHOTOIMAGING**

[75] Inventors: **Ludovicus Lucas Mertens,  
Borgerhout; Jozef Willy Van Den  
Houte, Berchem; Freddy Ghisleen  
Van Royen, Wommelgem, all of  
Belgium**

[73] Assignee: **Agfa-Gevaert N.V., Mortsel,  
Belgium**

[22] Filed: **Aug. 25, 1972**

[21] Appl. No.: **283,756**

[30] **Foreign Application Priority Data**

Aug. 27, 1971 Great Britain ..... 40349/71

[52] **U.S. Cl. .... 96/48 R, 96/48 QP, 96/45.2,  
96/90 PC, 96/90 R**

[51] **Int. Cl. .... G03c 5/24, G03c 1/52**

[58] **Field of Search .. 96/48 R, 45.2, 90 PC, 48 QP,  
96/90 R**

[56] **References Cited**

UNITED STATES PATENTS

|           |         |                       |          |
|-----------|---------|-----------------------|----------|
| 2,936,235 | 5/1960  | Chalkley .....        | 96/90    |
| 3,272,635 | 9/1966  | Sprague et al. ....   | 96/90    |
| 3,285,744 | 11/1966 | Sprague et al. ....   | 96/90    |
| 3,486,899 | 12/1969 | Brown.....            | 96/90 PC |
| 3,547,646 | 12/1970 | Hori et al. ....      | 96/90    |
| 3,558,317 | 1/1971  | Petro et al. ....     | 96/90    |
| 3,642,479 | 2/1972  | Van Allan et al. .... | 96/90 PC |
| 3,660,086 | 5/1972  | Tamai et al. ....     | 96/90 PC |

FOREIGN PATENTS OR APPLICATIONS

1,274,655 8/1968 Germany ..... 96/90 PC

Primary Examiner—Ronald H. Smith

Assistant Examiner—Won H. Louie, Jr.

Attorney, Agent, or Firm—William J. Daniel

[57] **ABSTRACT**

A photographic process wherein a visible image is formed in a recording material which comprises in intimate admixture:

1. at least one spiropyran compound,
2. at least one ultra-violet radiation-sensitive compound capable of producing on exposure with ultra-violet radiation with the spiropyran compound a dye salt, and in working relationship with said mixture an organic compound, which is an amido, acylamino or ureido compound corresponding to the following general formula:



wherein:

$R_1$  represents an organic group of the type present in a carboxylic acid chloride, a  $-NHR_3$  or a



group in which each of  $R_3$  and  $R_4$  represent an alkyl group or an aryl group, and  
 $R_2$  represents hydrogen, or an organic group.

**20 Claims, No Drawings**

PHOTOCROMIC MATERIAL CONTAINING A SPIROPYRAN COMPOUND, A POLYHALOGENATED HYDROCARBON PHOTOACTIVATOR AND AN ACETANILIDE SENSITIZER AND THE USE THEREOF IN PHOTOIMAGING

This invention relates to photographic recording and reproduction of information and to materials suited therefor.

The use of particular spiropyrans in the manufacture of photographic recording materials is known e.g. from the U.S. Pat. No. 2,953,454 of E. Berman — Nat. Cash Reg., issued Sept. 20, 1960. The spiropyrans described therein are characterized as being reversibly transformable into a coloured form by activating electromagnetic energy.

In many applications such reversible transformation is not desirable and therefore efforts have been made to obtain a print-out colour image, the colour of which does not fade by keeping it in the dark or by a further irradiation with electromagnetic radiation differing in wavelength from the radiation originally applied.

In the German Patent Specification No. 1,274,655 filed Dec. 15, 1965 by Telefunken Patentverwertungs G.m.b.H. a recording material has been described by means of which stable print-out dyestuff images can be obtained by using spiropyrans in admixture with a compound that activated with electromagnetic radiation can yield photolytically formed free radicals.

The starting substances for these radicals are preferably halogenated organic compounds.

The recording materials described in the latter Patent Specification need rather long exposure times with the conventional ultra-violet radiation sources.

It is an object of the present invention to provide a method for increasing the photosensitivity of recording materials containing a photosensitive compound that by information-wise exposure to activating electromagnetic radiation yields a dyestuff image by reaction with a spiropyran compound.

It is another object of the present invention to provide a method for making visible or intensifying a latent image or barely visible image produced with said spiropyran and photosensitive compound. Said method is

called hereinafter "optical development" for it operates with an overall exposure in the wavelength range of electromagnetic radiation absorbed by dyestuff traces formed in the image-wise exposure.

It is a further object of the present invention to provide photographic materials suited for use in said methods.

It has now been found that the photosensitivity for forming a directly visible image or optical development sensitivity of a recording material containing in intimate admixture:

1. at least one spiropyran compound, and
2. at least one ultra-violet radiation-sensitive compound capable of producing an exposure to ultraviolet radiation with said spiropyran compound a dyestuff salt, is increased by using in working relationship with said mixture an organic compound being: an amido, acylamino or ureido compound corresponding to the following general formula:



wherein:

$R_1$  represents an organic group e.g. of the type present in a carboxylic acid chloride e.g. an alkyl group, an aryl group or heterocyclic group including these groups in substituted form, or a  $-NHR_3$  or



group in which each of  $R_3$  and  $R_4$  represent an alkyl group or an aryl group e.g. a phenyl group including these groups in substituted form, and

$R_2$  represents hydrogen or an organic group e.g. an alkyl group, an aryl group e.g. phenyl group or a heterocyclic group including these groups in substituted form.

Preferred sensitizing agents according to the above general formula are acetanilide and acetanilide derivatives.

Examples of useful sensitizing agents according to the general formula are listed in the following Table 1.

TABLE 1

| Number of the Compound | Structural formula | Melting point (°C.) | Reference for preparation        |
|------------------------|--------------------|---------------------|----------------------------------|
| 1.....                 |                    | 150                 | Ber. 60, 219 (1927).             |
| 2.....                 |                    | 135                 | Arch. der Pharmazie (1926) 324.  |
| 3.....                 |                    | 166                 | Rec. Trav. Chim. 41, 659 (1922). |
| 4.....                 |                    | 147                 | Monatsh. 48, 128.                |
| 5.....                 |                    | 130                 | Ber. 42, 3103 (1909).            |

TABLE 1—Continued

| Number<br>of the<br>compound | Structural formula          | Melting<br>point<br>(° C.) | Reference for preparation                                                                    |
|------------------------------|-----------------------------|----------------------------|----------------------------------------------------------------------------------------------|
| 6-----                       |                             | 168                        | J. pr. Chem. [2] 84, 530 (1911).                                                             |
| 7-----                       |                             | 170                        | Annalen 260 234 (1890).                                                                      |
| 8-----                       |                             | 102                        | Ber. 21, 1159 (1888).                                                                        |
| 9-----                       |                             | 142                        | Ber. 33, 2643 (1900).                                                                        |
| 10-----                      |                             | 156                        | Ber. 16, 2003 (1883).                                                                        |
| 11-----                      |                             | 86                         | Helv. Chim. Acta 11, 779.                                                                    |
| 12-----                      |                             | 111                        | J. pr. Chem. [2] 84, 649 (1911).                                                             |
| 13-----                      |                             | 242                        | A. Vogel, Practical Organic Chemistry, Longmans, Green and Co., Ltd. London, 3rd Ed. p. 646. |
| 14-----                      |                             | 132                        | J. Chem. Soc. 1926, 8.                                                                       |
| 15-----                      | $\text{CH}_3\text{CO-NH}_2$ | 82                         |                                                                                              |
| 16-----                      |                             | 80-81                      | Am. Soc. 24, 763.                                                                            |

Spiropyran compounds suited for photographic image formation according to the present invention are spiropyrans containing at least one pyran ring having in the ortho- and meta-position to the oxygen atom a condensed benzo, naphtho or other higher aromatic polycyclic condensed ring system including these condensed rings or ring systems in substituted state e.g. an anthraceno or a phenanthreno ring system e.g. as present in a spirodibenzopyran, a spirodinaphthopyran, a spirobenzonaphthopyran, a trimethylindolinobenzospiropyran, a trimethylindolinonaphthospiropyran or such spiropyrans containing condensed aromatic nuclei of the anthracene or phenanthrene type.

In said spiropyrans the pyran rings, the condensed benzo, the condensed higher aromatic rings as well as the 1,3,3-trimethylindolino ring may be substituted.

Suitable substituents therefore are e.g. hydrocarbon groups such as alkyl groups, e.g. lower alkyl groups such as methyl, substituted alkyl groups e.g. halogen, or phenyl substituted alkyl groups, alkylene ester groups e.g. a  $-\text{CH}_2-\text{COOC}_2\text{H}_5$  group, alkylene carboxyl groups e.g. a  $-\text{CH}_2-\text{COOH}$  group, carbonamide groups or substituted carbonamide groups e.g. a



group, halogen, nitro, hydroxy, alkoxy, aryloxy or a substituent linking the carbon atoms in 3,3'-position in the spiropyran system together e.g. a  $(CH_2)_n$ -chain wherein n is 2 or 3.

General formulae covering particularly suited spiro-pyrans are the following:





5 group, or R<sub>1</sub> and R'<sub>1</sub> together represent a -(CH<sub>2</sub>)<sub>n</sub>—chain wherein n=2 or 3 to link the carbon atoms in the 3 and 3' positions.

10 Suited spiropyran compounds and their preparation are described in the published German Patent Applications 1,274,655 filed Dec. 15, 1965 by Telefunken Patentverwertungs G.m.b.H., 1,269,665, 1,286,110, 1,286,111 and 1,286,112 all filed Sept. 30, 1966 by Telefunken Patentverwertungs G.m.b.H., and by W. Dilthey, Berres, Holterhoff, Wubken, J.Pr.Ch. [2] 114, 187 (1926), by C. F. Koelsch and W. R. Workman in J.A.C.S. 74 6288 (1952) and in J.Chem.Soc. (1934), 1571 by I. M. Heilbron and G. F. Howard.

20 Preferred spiropyran compounds are spirodinaphthopyrans and spirobenzonaphthopyrans including such compounds wherein the naphtho- and/or benzo ring(s) is (are) substituted.

25 An illustrative list of particularly useful spiropyran compounds is given in the following Table 2.

TABLE 2

|        | Spiropyran compound | Melting point<br>(°C.) |
|--------|---------------------|------------------------|
| 1..... |                     | 257                    |
| 2..... |                     | 204                    |
| 3..... |                     | 208                    |
| 4..... |                     | 185                    |
| 5..... |                     | 164                    |
| 6..... |                     | 166                    |
| 7..... |                     | 210                    |

TABLE 2—Continued

| Spiropyran compound |  | Melting point<br>(° C.) |
|---------------------|--|-------------------------|
| 8.....              |  | 238                     |
| 9.....              |  | 140                     |
| 10.....             |  | 180                     |
| 11.....             |  | 260                     |
| 12.....             |  | >280                    |
| 13.....             |  | >280                    |
| 14.....             |  | >280                    |
| 15.....             |  | 168                     |
| 16.....             |  | 110                     |
| 17.....             |  | 163                     |
| 18.....             |  | 110                     |
| 19.....             |  | 185                     |

TABLE 2—Continued

|    | Spiropyran compound | Melting point<br>(°C.) |
|----|---------------------|------------------------|
| 20 |                     | 206                    |
| 21 |                     | 180                    |
| 22 |                     | 88                     |
| 23 |                     | >260                   |
| 24 |                     | 173                    |
| 25 |                     | 193                    |
| 26 |                     | 158                    |
| 27 |                     | 144                    |

TABLE 2—Continued

|    | Spiropyran compound                                                                 | Melting point<br>(°C.) |
|----|-------------------------------------------------------------------------------------|------------------------|
| 28 |    | 180                    |
| 29 |    | 160                    |
| 30 |   | 112                    |
| 31 |  | 120                    |
| 32 |  | ±200                   |
| 33 |  | 248                    |

TABLE 2—Continued

|         | Spiropyran compound | Melting point<br>(°C.) |
|---------|---------------------|------------------------|
| 34----- |                     | 182                    |
| 35----- |                     | 160                    |
| 36----- |                     | ±250                   |
| 37----- |                     | 173                    |
| 38----- |                     | 133                    |

TABLE 2—Continued

|         | Spiropyran compound | Melting point<br>(°C.) |
|---------|---------------------|------------------------|
| 39..... |                     | 146                    |

In order to illustrate in more details the preparation of the diarylo spiro-pyran compounds and the indolino-arylospiropyran compounds the following preparation receipts are given:

Preparation 1

Preparation of 3-methyldi-β-naphthospiropyran (compound 2 of Table 2)

In a 2 litre three-necked flask, fitted with a reflux condenser and a gas inlet tube reaching nearly the bottom of the flask are introduced:

|                            |                   |
|----------------------------|-------------------|
| ethanol                    | 1 litre           |
| butanone                   | 22 ml (0.25 mole) |
| 2-hydroxy-1-naphthaldehyde | 86 g (0.5 mole)   |

The flask is shaken until partial dissolution of the ingredients. Dry hydrogen chloride gas is introduced at a rate, which allows complete absorption and the start of ethanol reflux. Thereupon the already highly blue coloured mixture is cooled down in a mixture of ice and sodium chloride and the introduction of hydrogen chloride gas is continued until saturation. In the reaction mixture green crystals of pyrylium salt are formed and the crystallization is allowed to proceed overnight in a refrigerator.

The pyrylium salt formed is separated by suction, is washed with ethanol, and thereupon suspended in 300 ml of ethanol.

Whilst stirring a 10 percent by weight aqueous solution of ammonium hydroxide is added until the mixture is definitely alkaline. During this operation the mixture becomes colourless.

The obtained crystalline product is separated by suction, washed with water, and dried.

Finally the spiropyran compound is recrystallized from 600 ml of benzene, separated again, and dried under reduced pressure at 50°–60°C. Yield: 45 g. Melting point: 204°C.

Preparation 2

Preparation of 1,3,3-trimethylindolinobenzopyrylospiro (compound 22 of Table 2)

In a 100 ml flask fitted with a reflux condenser the following ingredients are introduced:

|                                        |                   |
|----------------------------------------|-------------------|
| salicylaldehyde                        | 3.7 g (0.03 mole) |
| 1,3,3-trimethyl-2-methylene indolamine | 5.1 g (0.03 mole) |
| ethanol                                | 90 ml             |

The solution is refluxed for 2 hours, whereupon the mixture is cooled and filtered.

Water is added to the filtrate. The solid is then sepa-

rated by suction, washed with water, and dried in vacuo.

The spiro compound is recrystallized from 15 ml of hexane.

Yield: 5 g. Melting point: 93°–94°C.

For use according to the present invention the compound capable of producing a dye salt with a spiropyran on exposure to activating electromagnetic radiation is preferably an organic polyhalogen compound, from which a halogen-containing radical can be separated photolytically. Compounds possessing this property are within the scope of the following general formula:



wherein:

each of A, B, X, and Y are halogen atoms of the group of chlorine, bromine, or iodine, or wherein one of said groups A, B, X, or Y represents an alkyl group, including a substituted alkyl group e.g. a halogen substituted alkyl group, a hydroxylalkyl group or an aralkyl group e.g. a benzyl group, an aryl group, a substituted aryl group or an aryl group and the other groups chlorine, bromine, or iodine, or wherein at least two of said groups A, B, X, or Y represent an aromatic acyl group e.g. a benzoyl group and the other groups chlorine, bromine, or iodine.

Suitable representatives falling within the scope of the general formula are organic halides such as carbon tetrabromide, bromoform, iodoform, hexachloroethane, hexahexabromoethane, pentabromoethane, 1,1,2,2-tetrabromoethane,  $\alpha$ ,  $\alpha$ ,  $\alpha$ -tribromoacetophenone, and tribromoethanol.

The amount of the sensitizing agent according to the above general formula may vary within a wide range depending on the intensity of the desired effect.

Preferred amounts of sensitizing agent are in the weight ratio range of 1:1 to 0.1:1 with respect to the spiropyran compound(s).

The spiropyran compound(s) are used preferably in admixture with a 5- to 20-fold amount by weight of photosensitive organic halogen compound such as carbon tetrabromide. This ratio, however, is not limitative since useful results can be obtained with e.g. the spiropyran and photosensitive polyhalogen compound in a ratio by weight in the range of 1:1 to 1:50.

A sensitizing agent of the above general formula may be used alone or in combination with one or more other

sensitizing compounds belonging to one of the following classes:

(A) organic compounds containing two groups of different electron-affinity (the term group includes group as well as atom) linked to each other through a conjugated system.

Useful sensitizing agents of class (A) are those having one of the following general formulae (I), (II), (III), (IV), (V) or (VI):



wherein:

D represents an electron-donating group e.g. an alkyl (preferably C<sub>1</sub>-C<sub>5</sub> alkyl), cycloalkyl or aralkyl substituted amino or hydroxy group, preferably a monoalkyl amino group, a dialkylamino group or an alkoxy group,

Z represents a conjugated system e.g. a polymethine chain or an azamethine chain including such chain that is substituted or makes part of a ring structure e.g. a phenylene or a naphthylene ring,

R represents hydrogen, a hydrocarbon group e.g. an alkyl, an aryl or a heterocyclic group preferably a methyl group or a phenyl group, or the necessary atoms to form a homocyclic or heterocyclic ring with an atom of the group Z,

Q<sub>1</sub> represents the non-metallic atoms necessary to complete a ring or ring system in which the group C=X through a conjugated system is linked to an electron-donating group as described for D,

X represents an electronegative atom or group e.g. oxygen, =N-R wherein R is hydrogen or an aromatic group, sulphur, selenium,



and other bivalent electron-attracting groups known in organic chemistry, preferably however X represents oxygen or sulphur,

Q<sub>2</sub> represents the non-metallic atoms necessary to complete a ring or ring system wherein the group



is linked through a conjugated system to an electron-attracting group e.g. a carbonyl group, a thi-

ocarbonyl group, a sulfonyl group or a dicyanomethylene group, or represents the atoms necessary to form with the carbon atom of the group



a heterocyclic ring having an electronegative character with respect to the group D e.g. a benzoxazole ring,

Y represents an electron-attracting group e.g.



or the group



wherein X has the same meaning as described above,

Q<sub>3</sub> represents a heterocyclic nucleus containing an electron-donating group e.g. a dialkylamino group that is linked through a conjugated system with the group



wherein P and Q each represent an electron-attracting substituent e.g. a cyano group or wherein P and Q together represent the atoms necessary to close a heterocyclic ring with electronegative character e.g. as present in merocyanine dyes such as a ketomethylene ring, the rhodanine nucleus being a specific example,

each of L<sub>1</sub> and L<sub>3</sub> represent a methine group or a substituted methine group, and

L<sub>2</sub> represents a monovalent chemical bond, an  $\alpha$ ,  $\beta$ -ethylenically unsaturated bivalent group e.g. a



group or a plurality of said groups linked to each other, or L<sub>1</sub>, L<sub>2</sub>, and L<sub>3</sub> together represent a double bond linking the group



to the group



Preferred compounds falling within the scope of formula (I) are:



Preferred compounds falling within the scope of formula (II) are:



Preferred compounds falling within the scope of formula (III) as described e.g. in the Belgian Patent Specification 747,849 filed March 23, 1970 by Gevaert-Agfa N.V. corresponding with the U.S. Pat. appl. Ser. No. 22,376. Representatives thereof are e.g.:



Preferred compounds falling within the scope of formula (IV) are styryl dye bases and styryl vinyl dye bases and compounds such as:



Ref. United States patent specification 2,793,792 of J. B. Pilkington, issued May 28, 1957.



(Ref. J. Prakt. Chem. [2], 157, p. 219 (1941)).



Ref. Ber. 89, p. 1748 (1956).



Ref. Ber. 89, p. 1748 (1956).



Ref. U.S. pat. spec. 3,189,447 of Wilhelm Mengenbauer, Martha Tomanek and Hans Behnenburg, issued June 15, 1965.



The N-vinyl polymers and copolymers can be prepared by application of one of the various known polymerization procedures, e.g., by pearl- or emulsion polymerization or by polymerization in solution, whereby the initiation of the polymerization can occur by free radicals, by ion formation, or by radiation e.g., with actinic light. It is to be noted that the polymerization degree is not critical and can vary between wide limits. As far as the copolymers are concerned, it is further to be noted that the content of groups corresponding to the general formula given hereinbefore is not critical and, as shown further on in the table of copolymers containing N-vinylcarbazole units, it can vary between wide limits, say, e.g. between 20 and 95 percent, taking into account the properties of the compounds used in the preparation of the copolymers and the required sensitizing and/or mechanical properties. In general, the best results are obtained with copolymers having a content of vinylcarbazole units between 40 and 90 %.

The preparation of suitable poly-N-vinylcarbazoles is described e.g. in the German Patent Specifications 931,731 filed Mar. 4, 1953, 936,421 filed Feb. 20, 1953, 1,097,680 filed Oct. 15, 1959 all three by B.A.S.F., and 1,158,367 filed July 18, 1962 by Gevaert Photo-Producten N.V., and the U.S. Pat. No. 2,072,465 of W. Reppe, E. Keyssner and E. Dorrer, issued March 2, 1937. The preparation of poly-N-vinylpyrrole proceeds analogously.

The preparation of suitable N-vinylcarbazole copolymers is described in the United Kingdom Patent Specification 964,875 filed April 21, 1960 by Gevaert Photo-Producten N.V. which specification also contains a preparation receipt for poly(N-allyl carbazole) ( $R_1 = \text{CH}_3$  and  $R_2 = \text{H}$ ) and for poly(N-propenyl carbazole) ( $R_1 = \text{H}$ ,  $R_2 = \text{H}$ ,  $A = -\text{CH}_2-$ ).

The poly-N-vinyl indoles are described in the published German Patent Application 1,906,831 filed Feb. 12, 1969 and 1,917,747 filed Apr. 5, 1969 by I.B.M. Corp. The polyN-vinyl diphenylamine is described in the published German Patent Application 2,007,692 filed Mar. 3, 1969 by Xerox corp. Halogen-substituted poly-N-vinyl carbazoles are described in the published Japanese Patent Applications 21,875/67 filed June 18, 1964, 25,230/67 filed Oct. 13, 1864, 7,592/68 filed Nov. 27, 1964, 19,751/67 filed June 18, 1964 and 7,591/68 filed Nov. 18, 1964 all by Matsushita Electric Industrial Co. Ltd.

For illustrative purposes suitable vinyl copolymers containing N-vinyl carbazole units are enumerated in the following table 2.

Table 2

| Copolymer                                                         | mole % of N-vinyl carbazole |
|-------------------------------------------------------------------|-----------------------------|
| copolymer of N-vinylcarbazole and vinylidene chloride             | 85.4                        |
| copolymer of N-vinylcarbazole and 3,3',5-trimethyl isononyl ether | 93                          |
| copolymer of N-vinylcarbazole and vinyl acetate                   | 88.6                        |
| copolymer of N-vinylcarbazole and isopropenyl acetate             | 94.5                        |
| copolymer of N-vinylcarbazole and vinyl stearate                  | 37.5                        |
| copolymer of N-vinylcarbazole and methyl acrylate                 | 67.6                        |
| copolymer of N-vinylcarbazole and ethyl acrylate                  | 41                          |
| graft copolymer of N-vinylcarbazole and ethyl-acrylate            | 90.3                        |
| emulsion polymer of N-vinylcarbazole and polyethylacrylate        | 94.5                        |
| copolymer of N-vinylcarbazole and n-butyl acrylate                | 58.3                        |

3,820,995  
24  
Table 2-Continued

| Copolymer                                                                                                    | mole % of N-vinyl carbazole |
|--------------------------------------------------------------------------------------------------------------|-----------------------------|
| 5 copolymer of N-vinylcarbazole and 2-ethyl hexylacrylate                                                    | 51.6                        |
| copolymer of N-vinylcarbazole and acryloxyethyl diethylamine                                                 | 76.6                        |
| copolymer of N-vinylcarbazole and vinyl cinnamate                                                            | 92.5                        |
| 10 copolymer of N-vinylcarbazole and methyl methacrylate                                                     | 62.7                        |
| copolymer of N-vinylcarbazole and isobutyl methacrylate                                                      | 51.8                        |
| copolymer of N-vinylcarbazole and lauryl methacrylate                                                        | 77.4                        |
| copolymer of N-vinylcarbazole and methylacryloxyethyl diethylamine                                           | 9.7                         |
| 15 copolymer of N-vinylcarbazole and acrylonitrile                                                           | 88                          |
| graft copolymer of N-vinylcarbazole and butylaldehyde acetal of polyvinylalcohol                             | 30                          |
| copolymer of N-vinylcarbazole and di(2-dichloroethyl)-vinyl phosphonate                                      | 82.4                        |
| copolymer of N-vinylcarbazole and styrene                                                                    | 49                          |
| 20 graft copolymer of N-vinylcarbazole and polystyrene                                                       | 27.3                        |
| copolymer of N-vinylcarbazole and vinyl naphthalene                                                          | 47.1                        |
| copolymer of N-vinylcarbazole and anthracene-(9,10)                                                          | 91.5                        |
| copolymer of N-vinylcarbazole and 2-vinylpyridine                                                            | 31.8                        |
| copolymer of N-vinylcarbazole and 4-vinylpyridine                                                            | 32.4                        |
| copolymer of N-vinylcarbazole and N-vinylpyrrolidine                                                         | 69.1                        |
| 25 terpolymer of N-vinylcarbazole, acrylonitrile and styrene                                                 | 20                          |
| graft copolymer of a terpolymer of vinyl chloride, vinyl acetate, and vinyl alcohol with N-vinylcarbazole    | 20.1                        |
| graft copolymer of a terpolymer of vinyl chloride, vinyl acetate, and maleic anhydride with N-vinylcarbazole | 55.1                        |

30

A preferred photosensitive recording material according to the present invention contains the spiropyran compound(s) and poly-N-vinylcarbazole in a ratio by weight within the range of 80:100 to 10:100.

The poly-N-vinylcarbazole is further preferably used in admixture with carbon tetrabromide or iodoform or a mixture of both of said polyhalogen compounds. Said polyhalogen compounds are preferably used with respect to poly-N-vinylcarbazole in a ratio by weight in the range of 160:100 to 20:100.

D. organic nitrogen containing compounds having a thiol group or in their tautomeric form a thione group as represented in the following tautomeric structural parts:



Preferred organic nitrogen containing compounds 50 are within the scope of the following tautomeric general formulae:



wherein:

X represents oxygen, sulphur, selenium or the group —NR in which R is hydrogen or an organic group e.g. an alkyl group including a substituted alkyl group, preferably a  $\text{C}_1\text{--}\text{C}_5$ -alkyl group, and

Z represents the atoms necessary to close a 5- or 6-membered heterocyclic nitrogen-containing ring or ring system including such ring or ring system in substituted form e.g. a benzthiazole, benz-selenazole, benzoxazole, or benzimidazole ring.

Particular examples of useful sensitizing agents of class (D) are:



phenyl stibine are with respect to photosensitive carbon tetrabromide and/or iodoform within the weight ratio range of 1:100 to 2.5:100.

A dry photographic coating containing the above mentioned ingredients may be formed by dissolving the binding agent(s) in a suitable inert solvent acting as dispersing or dissolving medium for the other ingredients and which is removed from the coating composition by evaporation, thus leaving a solid photographic recording layer on a properly chosen support. The supports may be of any kind used in silver halide photographic materials e.g. paper and film supports.

In order to realize the highest sensitivity, it is desirable to coat the recording layers in the absence of oxygen or to keep them before the exposure in an oxygen-free environment.

The photosensitive organic polyhalogen compounds that in exposed state form with a spiropyran compound a dyestuff salt normally are sensitive only in a wavelength range between 400 and 250 nm.

The recording materials of the present invention containing spirodiarylopyrans and the sensitizing agents of the general formula show especially in combination with polymers and copolymers containing N-vinylcarbazole units and serving as binding agent a remarkable high white and more particularly red light sensitivity. This unexpectedly high sensitivity in the visible spectrum range is increased yet, when during the visible light exposure the temperature of the recording layer composition is raised above 40°C. A very suitable operating temperature is in the range of 40°-70°C.

By the combination of the sensitizing agents of the general formula with organic spectral sensitizing dyes e.g. those of class (A) it is possible to further increase the spectral sensitivity in the visible spectrum and to obtain synergistic sensitizing effects.

On using a recording material containing superposed recording layers sensitized respectively in the red, green, and blue region of the spectrum and containing the proper dye-forming combination superposed cyan, magenta, and yellow separation images can be produced that offer a full reproduction of the multicolor original used in the information-wise exposure.

The recording materials sensitized according to the present invention are suited to product print-out images of different colour depending on the type of spiropyran compound used.

The stabilisation of the obtained prints may proceed by washing out the residual free radical generator with a suitable solvent or solvent mixture e.g. a hydrocarbon liquid such as petroleum ether optionally mixed with acetone, or by simply evaporating it by raising the temperature when the compound involved is sufficiently volatile. For the latter purpose and the high photosensitivity, carbon tetrabromide or a mixture of carbon tetrabromide and iodoform is preferred.

According to a preferred recording and reproduction process of the present invention the information-wise exposure is carried out in such a way that first a latent image is produced, which is transformed into a visible dye image by means of a so-called "optical development."

The optical development proceeds by exposing the recording layer containing the latent or barely visible image over its entire surface to visible radiation, which lies in the spectral absorption band of the products formed by the image-wise exposure and image-wise in-

teraction of the photoexposed ingredients (1) and (2) of the above-mentioned photosensitive composition. In the overall exposure no exposure light is used, to which the photosensitive polyhalogen compound is inherently sensitive since thereby the effect of the image-wise exposure would be masked by an overall colouration. It is advantageous to use in the optical development exposure a filter absorbing all the light corresponding with the wavelength range that is inherently absorbed by the ingredients of the non-Previously exposed recording layer.

The optical development effect is speeded up markedly and the image density is increased by applying heat e.g. supplied by contact with a hot body or through infrared radiation during the overall exposure to visible light.

The optical development speed obtains a particularly high value by the use of poly-N-vinylcarbazole or the copolymers containing N-vinyl carbazole units in combination with the present amido, acylamino, or ureido compounds. The addition of a triarylstibine such as triphenylstibine to this combination intensifies the image density obtained by the optical development procedure.

It is assumed that during the exposure applied in the optical development at least a part of the overall applied light energy is visible light absorbed by a dyestuff salt having the pyrylium structure when a diarylo spiropyran is used, or having an indolinium salt structure, when an indoline-arylospiropyran is used. Said salt seems to act as a spectral sensitizing agent for a chemical reaction between the photosensitive polyhalogen compound or radicals formed therefrom and the spiropyran.

In a preferred composition for forming print out as well as optically developable prints a mixture of carbon tetrabromide and iodoform yielding a superadditive sensitivity effect is used.

According to an alternative embodiment of the optical development technique the recording material is first overall exposed to electromagnetic radiation to produce non-differentially over the whole recording layer latent dyestuff centres that afterwards are optically developed information-wise by a sufficiently strong information-wise exposure in the absorption band of the dyestuff centres. Optionally the information-wise exposure proceeds simultaneously with an overall heating e.g. effected by an overall infra-red radiation exposure.

Instead of applying an overall pre-exposure to form the dyestuff centres these dyestuffs may be added e.g. applied by imbibition (diffusion) in minor amounts to the recording layer composition to act as optical development nuclei for the dye image formation by image-wise exposure.

According to a special embodiment the spiropyrans are formed in the non-exposed recording layer composition "in situ" by starting from the corresponding pyrylium and indolinium salts and adapting the pH in a proper way to obtain the spiropyrans that may be considered as the dyestuff precursors of the pyrylium and indolinium salts, respectively.

The information-wise exposure applied in the present invention may be a contact exposure of the direct or reflex type and likewise an optical projection exposure as used e.g. in an optical enlarging apparatus. The in-

formation-wise exposure need not be simultaneous in all parts of the recording material. The exposure may be progressive in one continuous step as e.g. in sound track recording or in successive intermittent steps provided the required information-wise change is obtained. Thus the recording material may be scanned with an image-wise modulated radiant energy spot of high intensity e.g. a laser beam, or the material may be progressively exposed through a slit, e.g. is exposed to copying light of a tubular lamp that is given a translation movement along the original.

A recording material of the present invention being suited for the recording of information in the form of modulated ultraviolet radiation can be used in X-ray and electron-beam recording. X-ray beams can be absorbed in high energy absorbing substances and create by means of them so-called secondary photons e.g. of the ultraviolet radiation energy band and photoelectrons that are absorbed by the photosensitive polyhalogen compound forming through its photoradicals a dyestuff salt with the spiropyran. Substances for high energy absorption that may be incorporated in the recording element contain the elements lead, mercury, bismuth, barium and/or tungsten. Lead compounds that themselves are photosensitive are preferred e.g. lead monoxide, lead bromide and lead iodide.

Suitable light sources for use in a recording method of the present invention are ultra-violet radiation sources, xenon-gas lamps, incandescent bulbs, sunlight and flash lamps. In the overall exposure for the optical development an infra-red lamp emitting also in the visible spectrum is used preferably.

Electron beam and laser beam recording proceed with the apparatus suited for that purpose and known to those skilled in the art.

Recording materials of the present invention are very versatile in that by the use of a proper sensitizing agent they can be applied to continuous tone or halftone reproduction. They can offer very contrasty images so that they are very suited for the reproduction of line and screen type originals and find a successful use in a great variety of graphic art applications. Due to the very high resolving power of the recording materials (the dyestuffs are formed in molecularly divided form) the recording materials of the present invention are particularly suited for microfilm reproduction and high precision image rendering as e.g. in the production of optical micromask masters used in the manufacturing of microelectronic circuitry.

The reflex-exposure properties of the present recording materials make them very useful in the field of document reproduction since in a reflex-contact exposure they offer print-out images of a sufficiently intense spectral density.

According to a special application a recording layer as described herein is used in conjunction with a magnetic recording layer and is more particularly applied to the rear side of a flexible tape support carrying the magnetic recording layer. By the use of such a material a sound track is formed in the magnetic recording layer and a visual text image corresponding with the sound track is photographed on the recording layer of the present invention.

Such a recording material thus allows the storing of optical and acoustic signals and the reproduction of both informations simultaneously.

The present invention is illustrated by the following

examples without, however, limiting it thereto. The percentages are by weight unless otherwise indicated.

#### EXAMPLE 1

##### Preparation of sample A

A mixture of 120 mg of carbon tetrabromide, 120 mg of iodoform, 100 mg of 3-methyl-di- $\beta$ -naphthospiropyran and 8 ml of a 5 percent solution of polystyrene in methylene chloride was coated at a thickness of 0.1 mm onto a non-subbed polyethylene terephthalate support.

The coating was dried in the dark at room temperature.

##### Preparation of sample B

A mixture of 120 mg of carbon tetrabromide, 120 mg of iodoform, 100 mg of 3-methyl-di- $\beta$ -naphthospiropyran, 60 mg of acetanilide, and 8 ml of a 5 % solution of polystyrene in methylene chloride was coated on a non-subbed polyethylene terephthalate support.

The coating was dried in the dark at room temperature.

##### Print-out processing of samples A and B

The samples A and B were exposed through a grey wedge with a constant of 0.15 by means of a 1000 W mercury vapour bulb placed at a distance of 5 cm.

In the following table the exposure times and the number of directly reproduced wedge print steps is mentioned.

Table

|    | Exposure time<br>sec. | Amount of reproduced steps |          |
|----|-----------------------|----------------------------|----------|
|    |                       | Sample A                   | Sample B |
| 35 | 20                    | 10                         | 16       |
|    | 5                     | 6                          | 9        |
|    | 2                     | 0                          | 5        |

40 By carrying out the contact-exposure in a 3M PHOTOCOPIER 179 (copying apparatus marketed by Minnesota Mining and Manufacturing Co., St. Paul, Minn., U.S.A.) operating at full intensity for an exposure time of 30 sec 0 steps were reproduced with sample A and 45 2 steps with sample B. The temperature of the recording materials during their exposure was about 50°C.

The image obtained was stabilized by heating the recording material for 1 min. at 140°C.

#### EXAMPLE 2

##### Preparation of sample A

A mixture of 120 mg of carbon tetrabromide, 120 mg of iodoform, 100 mg of 3-methyl-di- $\beta$ -naphthospiropyran, 20 mg of triphenylstibine, and 8 ml of a 5 % solution of poly-N-vinylcarbazole in methylene chloride was coated at a thickness of 0.1 mm on a non-subbed polyethylene terephthalate support.

##### Preparation of Sample B

60 A mixture of 120 mg of carbon tetrabromide, 120 mg of iodoform, 100 mg of 3-methyl-di- $\beta$ -naphthospiropyran, 20 mg of triphenylstibine, 60 mg of acetanilide, and 8 ml of a 5 percent poly-N-vinylcarbazole solution in methylene chloride was coated at a thickness of 0.1 mm on a non-subbed polyethylene terephthalate support.

The coating was dried in the dark at room temperature.

## Print-out processing of samples A and B

The samples A and B were exposed in contact through a grey wedge with constant 0.15 in a 3M PHOTOCOPIER 179 (trade name). The exposure lasted 30 sec and the temperature of the recording materials during their exposure was about 50°C.

On the sample A a wedge print with 4 visible steps and on sample B a wedge print with 12 visible steps was reproduced.

The same recording materials were used for the production of print-out images by means of a diazo copying apparatus marketed under the name ACTINA SH by La Cellophane, Paris, France, and operating with the ultraviolet radiation source of 1000 W.

In the following table the exposure times and the number of directly reproduced wedge print steps is mentioned.

Table

| Exposure time<br>sec. | Amount of reproduced steps |          |
|-----------------------|----------------------------|----------|
|                       | Sample A                   | Sample B |
| 20                    | 14                         | 19       |
| 5                     | 8                          | 15       |
| 2                     | 5                          | 9        |

The stabilization of the images was carried out by heating the recording material for 1 min. at 180°C.

## EXAMPLE 3

## Preparation of the recording materials for comparative testing.

120 mg of carbon tetrabromide, 120 mg of iodoform, 100 mg of 3-methyl-di- $\beta$ -naphthospiro-*pyran*, 30 mg of triphenylstibine, and 60 mg of a sensitizing agent indicated by number in the description in Table 1 are dissolved in 8 ml of a 5 percent solution of poly-N-vinylcarbazole in methylene chloride.

The solutions are coated at a thickness of 0.1 mm. The recording layers were dried at room temperature in the dark and exposed for 30 sec. in contact with a grey wedge (constant 0.15) in a 3M PHOTOCOPIER 179 (trade name). The temperature of the exposed recording material was about 50°C.

In the following table the number of wedge print steps obtained on the different materials is listed.

Table

| Number of sensitizing compound of general formula (I) | Number of reproduced steps |
|-------------------------------------------------------|----------------------------|
| — (blank)                                             | 4                          |
| 1                                                     | 12                         |
| 2                                                     | 11                         |
| 4                                                     | 8                          |
| 7                                                     | 13                         |
| 10                                                    | 12                         |
| 11                                                    | 10                         |
| 12                                                    | 11                         |
| 13                                                    | 9                          |
| 14                                                    | 9                          |
| 15                                                    | 8                          |
| 16                                                    | 13                         |

The stabilization of the images was carried out by heating the recording materials for 1 min. at 180°C.

## EXAMPLE 4

A mixture of 120 mg of carbon tetrabromide, 120 mg of iodoform, 100 mg of 3-methyl-di- $\beta$ -naphthospiro-

*pyran*, 30 mg of triphenylstibine, 60 mg of p-isopropylacetanilide and 8 ml of a 5 percent solution of poly-N-vinylcarbazole in methylene chloride were coated at a thickness of 0.1 mm on a non-subbed polyethylene terephthalate support. The resulting layer was dried at room temperature in the dark.

The recording layer was exposed through a transparent line original in a 3M PHOTOCOPIER 179 (trade name) operating at full intensity for an exposure time of 5 sec. The density of the obtained image was about 1.

The image was stabilized by treating the recording material in a solution consisting of toluene, acetone, n-hexane (1:1:4 parts by volume).

## EXAMPLE 5

A mixture of 120 mg of carbon tetrabromide, 120 mg of iodoform, 100 mg of 3-methyl-di- $\beta$ -naphthospiro-*pyran*, 60 mg of acetanilide, 20 mg of triphenylstibine was dissolved in 8 ml of 5 percent poly-N-vinylcarbazole solution in methylene chloride.

The solution was coated at a thickness of 0.1 mm on a non-subbed polyethylene terephthalate support. The coated layer was dried in the dark at room temperature.

## Print-out processing

The recording material was exposed in a 3M PHOTOCOPIER 179 (trade name) through a step wedge of constant 0.15. The exposure lasted 30 sec and yielded a print-out image containing 11 visible steps.

## Optical development processing

The recording material was exposed in the way described for the print-out processing but through a transparent line original and with an exposure time of only 2 sec, whereby no directly visible image was obtained.

The image-wise exposed recording layer was then overall exposed with a 250 W-infra-red lamp placed at a distance of 20 cm and irradiating the recording layer for 25 sec through a narrow band filter mainly transmitting light in the wavelength range of 600-610 nm.

The density of the cyan image obtained was above 1.

## EXAMPLE 6

A mixture of 300 mg of carbon tetrabromide, 100 mg of iodoform, 100 mg of 3-methyl-di- $\beta$ -naphthospiro-*pyran*, 30 mg of triphenylstibine, 60 mg of phenacetine, 5 mg of thio Michler's ketone, and 8 ml of a 5% poly-N-vinylcarbazole solution in methylene chloride was coated at a thickness of 0.1 mm on a non-subbed polyethylene terephthalate support. The resulting layer was dried in the dark at room temperature.

The dry recording layer was exposed for 3 sec through a transparent line original in a 3M PHOTOCOPIER 179 (trade name). A print-out image of neutral colour tone with a density above 1 was obtained.

## EXAMPLE 7

A mixture of 120 mg of carbon tetrabromide, 120 mg of iodoform, 100 mg of 3-methyl-di- $\beta$ -naphthospiro-*pyran*, 60 mg of acetanilide, 30 mg of triphenylstibine, and 8 ml of a 5 percent solution of poly-N-vinylcarbazole was coated at a thickness of 0.1 mm on a polyethylene terephthalate support. The layer was dried at room temperature in the dark.

The recording material obtained was divided up into 6 strips, which were exposed with a 100 W incandescent lamp placed at a distance of 15 cm. During the exposure the strips were kept at different temperatures in order to have an idea about the influence of heat during the exposure. In the following table the temperatures and corresponding exposure times for reaching a density (D) = 1 are mentioned.

Table

| Temperature °C | Exposure time (sec) for reaching (D) = 1 |
|----------------|------------------------------------------|
| 37             | 10                                       |
| 48             | 6                                        |
| 55             | 3                                        |
| 63             | 1                                        |
| 70             | 3                                        |

We claim:

1. A photographic process for forming a visible image in a recording material which comprises in intimate admixture:

1. at least one spiropyran compound of the group consisting of a spirodibenzopyran, a spirodinaphthopyran, a spirobenzonaphthopyran, a 1,3,3-trimethylindolinobenzospiropyran, a 1,3,3-trimethylindoline-naphthospopyran, or a spiropyran that contains a condensed aromatic nucleus of anthracene or phenanthrene,
2. at least one ultra-violet radiation-sensitive compound capable of producing on exposure with ultra-violet radiation with the spiropyran compound a dye salt and having the general formula



wherein:

each of A, B, X and Y is a chlorine, bromine, or iodine atom, or

one of said groups A, B, X or Y is an alkyl group, an aryl group or an aroyl group and the other groups are each chlorine, bromine, or iodine, or two of said groups A, B, X or Y each is an aromatic acyl group and the other groups chlorine, bromine, or iodine,

and in working relationship with said mixture an organic compound, which is an amido, acylamino or ureido compound corresponding to the following general formula:



wherein:

R<sub>1</sub> is an alkyl group, an aryl group, or a —NHR<sub>3</sub> or a



group in which each of R<sub>3</sub> and R<sub>4</sub> is an alkyl group or an aryl group, and

R<sub>2</sub> represents hydrogen, or an alkyl or aryl group, said process comprising the steps of imagewise exposing said recording material to activating electromagnetic radiation of an intensity sufficient to produce a visible image directly or a latent image that can be rendered visible by optical development.

2. The process of claim 1 wherein said exposure produces a latent image and said latent image is optically developed and comprising the steps of: imagewise exposing the recording material to activating electromagnetic radiation of an intensity sufficient to bring about a latent or barely visible image having an increased spectral sensitivity in a wavelength range outside the inherent sensitivity range of the ultra-violet light-sensitive compound, and then uniformly exposing the entire imagewise exposed recording material to light within the wavelength range for which the initially exposed portions are of increased sensitivity relative to the initially non-exposed portions, thereby increasing the visibility of said initially formed image.

3. The process of claim 1 wherein said exposure produces a latent image and said latent image is optically developed and comprising the steps of: uniformly exposing the entire recording material to electromagnetic radiation of an intensity sufficient to bring about in the recording material an increase in its spectral sensitivity in a wavelength range outside the inherent sensitivity range of the ultra-violet light-sensitive compound, and then imagewise exposing the overall exposed recording material within the wavelength range for which the overall exposed recording material is of increased sensitivity to increase the visibility of the initially formed image.

4. A photographic process according to claim 1 wherein said spiropyran compound corresponds to one of the following general formulae:





wherein:

R, R<sub>1</sub>, R'<sub>1</sub>, R<sub>2</sub>, R'<sub>2</sub>, R<sub>3</sub> and R'<sub>3</sub> each represent hydrogen, alkyl, alkyl substituted with halogen, alkyl substituted with an ester group, alkyl substituted with a carboxyl group, alkyl substituted with a N-phenylcarbamyl group, a hydroxy group, an alkoxy group, an aryloxy group, a phenyl group, piperidyl, acetyl, halogen, nitro, or R<sub>1</sub> and R'<sub>1</sub> together represent a -(CH<sub>2</sub>)<sub>n</sub>-chain wherein n = 2 or 3 to link the carbon atoms in the 3 and 3' positions together.

5. A process according to claim 1 wherein said mixture is used in combination with at least one sensitizing compound of the following classes.

A. an organic compound containing two radicals of different electron-affinity linked to each other through a conjugated system, and having one of the following general formulae (I), (II), (III), (IV), (V) or (VI):



35  
40

50

55

60

65

wherein:

D represents an electron-donating group selected from an amino group substituted with alkyl, cy-

cloalkyl or aralkyl, a hydroxy group or a hydroxy group substituted with alkyl, cycloalkyl or aralkyl,

Z represents a polymethylene chain, an azamethylene chain, phenylene or naphthalene,

R represents hydrogen, an alkyl group, an aryl group or the necessary atoms to form a homocyclic or heterocyclic ring with an atom of the group Z,

Q<sub>1</sub> represents the non-metal atoms necessary to complete a ring or ring system in which the group C=X is linked through a conjugated system of methine groups or of a chain of methine groups bound to nitrogen to a group D,

X represents an electronegative atom or group being selected from the group consisting of oxygen, =N-R wherein R is hydrogen or an aromatic group, sulphur, selenium, or



Q<sub>2</sub> represents the necessary atoms to form with the carbon atom of the group



a heterocyclic ring having an electronegative character with respect to the group D,

Y represents an electron-attracting group selected from the group consisting of



or the group



wherein X has the above meaning,

Q<sub>3</sub> represents a heterocyclic nucleus, containing an alkylamino group,

P and Q each represent an electron-attracting cyano group, or P and Q together represent the necessary atoms to close a heterocyclic ring with electronegative character, each of L<sub>1</sub>-L<sub>3</sub> represent a methine group, and L<sub>2</sub> represents a monovalent chemical bond, a



group or a

plurality of such groups linked to each other, or L<sub>1</sub>, L<sub>2</sub> and L<sub>3</sub> represent together a double bond linking the group



to the group



B. organic compounds containing an aromatic ring having two adjacent carbon atoms thereof in common with an adjacent ring free of conjugation, said adjacent ring at one end being linked to said aromatic ring through a carbon-carbon bond and at the other end is linked to said ring through an electron-donating group and having one of the following structural formulae:



wherein:

n is a positive integer of at least 2, and  
R is hydrogen or an alkyl group;

(C) polymeric compounds containing recurring units of the following general structure:



wherein:

Z represents a sulphur atom or a single bond,  
A represents a single bond or a divalent hydrocarbon group,

R<sub>1</sub> represents hydrogen or a lower alkyl group,  
R<sub>2</sub> represents hydrogen or a lower alkyl group,  
Q<sub>1</sub> and Q<sub>2</sub> each represent a hydrogen atom or together the necessary atoms to close an adjacent carbocyclic nucleus,

Q<sub>3</sub> and Q<sub>4</sub> each represent a hydrogen atom or together the necessary atoms to close an adjacent carbocyclic nucleus, and

n represents 1 or 2;

D. a tautomeric organic nitrogen containing compound corresponding to the following general formula:



in which: X represents oxygen, sulphur, selenium or the group



in which R is hydrogen, or an alkyl, allyl, or phenyl group, and

Z represents the necessary atoms to close a 5- or 6-membered heterocyclic nitrogen-containing ring system, and

E. an inorganic photoconductive metal compound in which said metal is zinc or lead.

6. A photographic process according to claim 1, wherein the recording material after the formation of

a visible image is uniformly heated to bring about image stabilisation.

7. A process according to claim 1, wherein R<sub>1</sub> is methyl in said organic compound.

8. A process according to claim 1, wherein said ultra-violet radiation-sensitive compound is carbon tetrabromide, iodoform, or a mixture thereof.

9. A process according to claim 1, wherein the recording material contains as anti-fogging agent at least one of a triaryl compound of a group V element or a sterically hindered phenol.

10. A process according to claim 1, wherein the mixture includes at least one binding agent, selected from the group of polymers and copolymers comprising styrene, vinyl acetate, acrylonitrile, acrylic acid ester, methacrylic acid ester, N-vinylcarbazole or butadiene units, a hydrophobic cellulose derivative, a phenoxy resin or a polycondensate of the polyester type including a polycarbonate resin.

11. A photosensitive recording material for the direct production of a visible image by imagewise exposure to activating electromagnetic radiation which comprises a layer of an intimate mixture consisting essentially of:

1. 1. at least one spiropyran compound of the group consisting of a spirodibenzopyran, a spirodinaphthopyran, a spirobenzonaphthopyran, a 1,3,3-trimethylindolinobenzospiropyran, a 1,3,3-trimethylindolino-naphthospopyran, or a spiropyran that contains a condensed aromatic nucleus of anthracene or phenanthrene,

2. at least one ultra-violet radiation-sensitive compound capable of producing on exposure with ultra-violet radiation with the spiropyran compound a dye salt and having the general formula



40 wherein: each of A, B, X and Y is a chlorine, bromine, or iodine atom, or each of said groups A, B, X or Y is an alkyl group, an aryl group or an aroyl group and the other groups are each chlorine, bromine, or iodine, or two of said groups A, B, X or Y each is an aromatic acyl group and the other groups chlorine, bromine, or iodine,

45 and in working relationship with said mixture an organic compound, which is an amido, acylamino or ureido compound corresponding to the following general formula:



55 wherein:

R<sub>1</sub> is an alkyl group, an aryl group, or a -NHR<sub>3</sub> or a



group in which each of R<sub>3</sub> and R<sub>4</sub> is an alkyl group or an aryl group, and

R<sub>2</sub> represents hydrogen, or an alkyl or aryl group.

12. A photosensitive recording material according to claim 11, wherein said spiropyran compound corresponds to one of the following general formulae:

39



wherein:

R, R<sub>1</sub>, R'<sub>1</sub>, R<sub>2</sub>, R'<sub>2</sub>, R<sub>3</sub> and R'<sub>3</sub> each represent hydrogen, alkyl, alkyl substituted with halogen, alkyl substituted with an ester group, alkyl substituted with a carboxyl group, alkyl substituted with a N-phenylcarbamyl group, a hydroxy group, an alkoxy group, an aryloxy group, a phenyl group, piperidyl, acetyl, halogen, nitro, or R<sub>1</sub> and R'<sub>1</sub> together represent a  $-(CH_2)_n-$  chain wherein  $n = 2$  or 3 to link carbon atoms in the 3 and 3' positions together.

13. A photosensitive recording material according to claim 11 wherein the recording material in addition to said mixture contains at least one compound belonging to one of the following classes:

A. an organic compound containing two radicals of different electron-affinity linked to each other through a conjugated system, and having one of the following general formulae (I), (II), (III), (IV), (V) or (VI):



(I) 65

(II)

(III)

40



wherein:

D represents an electron-donating group selected from an amino group substituted with alkyl, cycloalkyl or aralkyl, a hydroxy group or a hydroxy group substituted with alkyl, cycloalkyl or aralkyl,

Z represents a polyméthine chain, an azamethine chain, phenylene or naphthalene,

R represents hydrogen, an alkyl group, an aryl group or the necessary atoms to form a homocyclic or heterocyclic ring with an atom of the group Z,

Q<sub>1</sub> represents the non-metal atoms necessary to complete a ring or ring system in which the group C=X is linked through a conjugated system of methine groups or of a chain of methine groups bound to nitrogen to a group D,

X represents an electronegative atom or group being selected from the group consisting of oxygen, =N—R wherein R is hydrogen or an aromatic group, sulphur, selenium, or



Q<sub>2</sub> represents the necessary atoms to form with the carbon atom of the group



a heterocyclic ring having an electronegative character with respect to the group D,

Y represents an electron-attracting group selected from the group consisting of



or the group



wherein X has the above meaning,

Q<sub>3</sub> represents a heterocyclic nuclus, containing an alkylamino group,

P and Q each represent an electron-attracting cyano group, or P and Q together represent the necessary atoms to close a heterocyclic ring with electronegative character, each of L<sub>1</sub> and L<sub>3</sub> represent a methine group, and

$L_2$  represents a monovalent chemical bond, a



group or a

plurality of such groups linked to each other, or  $L_1$ ,  $L_2$  and  $L_3$  represent together a double bond linking the group



to the group



B. organic compounds containing an aromatic ring having two adjacent carbon atoms thereof in common with an adjacent ring free of conjugation, said adjacent ring at one end being linked to said aromatic ring through a carbon-carbon bond and at the other end is linked to said ring through an electron-donating group and having one of the following structural formulae:



wherein:

$n$  is a positive integer of at least 2, and  
 $R$  is hydrogen or an alkyl group;

C. polymeric compounds containing recurring units of the following general structure:



wherein:

$Z$  represents a sulphur atom or a single bond,  
 $A$  represents a single bond or a divalent hydrocarbon group,  
 $R_1$  represents hydrogen or a lower alkyl group,  
 $R_2$  represents hydrogen or a lower alkyl group,  
 $Q_1$  and  $Q_2$  each represent a hydrogen atom or to-

gether the necessary atoms to close an adjacent carbocyclic nucleus,

$Q_3$  and  $Q_4$  each represent a hydrogen atom or together the necessary atoms to close an adjacent carbocyclic nucleus, and.

$n$  represents 1 or 2;

D. a tautomeric organic nitrogen containing compound corresponding to the following general formula:



15 in which:  $X$  represents oxygen, sulphur, selenium or the group



in which  $R$  is hydrogen, or an alkyl, allyl, or phenyl group, and

$Z$  represents the necessary atoms to close a 5- or 6-membered heterocyclic nitrogen-containing ring system, and

20 E. an inorganic photoconductive metal compound in which said metal is zinc or lead.

14. A photosensitive recording material according to claim 13, wherein said material contains said mixture in layer form and includes poly-N-vinylcarbazole or a copolymer containing N-vinyl carbazole units as the sole binding agent therefor.

25 15. A photosensitive recording material according to claim 11, containing as an antifogging agent at least one of a triaryl compound of a group V element or a sterically hindered phenol.

30 16. A photosensitive recording material according to claim 11, wherein the recording material contains the spiropyran compound in admixture with a 1 to 50-fold amount by weight of the photosensitive organic polyhalogen compound.

35 17. A photosensitive recording material according to claim 14, wherein the recording material contains such spiropyran compound and poly-N-vinylcarbazole in a ratio by weight within the range of 80:100 to 10: 100.

40 18. A photosensitive recording material according to claim 17, wherein the organic polyhalogen compound is photosensitive carbon tetrabromide, iodoform, or a mixture thereof present with respect thereof present said poly-N-vinylcarbazole in a ratio by weight in the range of 160:100 to 20:100.

45 19. A photosensitive recording material according to claim 11 wherein  $R_1$  is methyl in said organic compound.

50 20. A photosensitive recording material according to claim 11, wherein said ultraviolet radiation-sensitive compound is carbon tetrabromide, iodoform, or a mixture thereof.

\* \* \* \* \*

UNITED STATES PATENT OFFICE  
CERTIFICATE OF CORRECTION

Patent No. 3,820,995

Dated June 28, 1974

Inventor(s) Ludovicus Lucas MERTENS et al

It is certified that error appears in the above-identified patent and that said Letters Patent are hereby corrected as shown below:

Column 35, Claim 4, lines 1-5, and Column 39, Claim 12, lines 17-21, correct the formula to read:



Column 39, Claim 12, lines 30-35, same as above.

Column 35, Claim 4, lines 15-20, correct the formula to read:



Column 39, Claim 12, lines 30-35, same as above.

Column 35, Claim 5, line 46, change "=Z" to -- =X -- (Formula I)

Column 39, Claim 13, line 63, same as above.

Column 42, Claim 13, line 22, correct the spelling of "close".

Signed and sealed this 26th day of November 1974.

(SEAL)

Attest:

McCOY M. GIBSON JR.  
Attesting Officer

C. MARSHALL DANN  
Commissioner of Patents